

F. I. DU PONT.  
SMOKELESS SHOTGUN POWDER.  
APPLICATION FILED MAY 28, 1919.

1,397,042.

Patented Nov. 15, 1921.

FIG. 1.



FIG. 2.



FIG. 3.

INVENTOR

Francis I. duPont  
BY  
Frankl. Busser  
ATTORNEY.

WITNESS:

John R. Kitchel.

# UNITED STATES PATENT OFFICE.

FRANCIS I. DU PONT, OF WILMINGTON, DELAWARE.

## SMOKELESS SHOTGUN-POWDER.

1,397,042.

Specification of Letters Patent. Patented Nov. 15, 1921.

Application filed May 28, 1919. Serial No. 300,266.

To all whom it may concern:

Be it known that I, FRANCIS I. DU PONT, a citizen of the United States, residing at Wilmington, county of New Castle, and 5 State of Delaware, have invented a new and useful Improvement in Smokeless Shotgun-Powder, of which the following is a full, clear, and exact description, reference being had to the accompanying drawings, which 10 form a part of this specification.

A known process of manufacturing smokeless shot gun powder of the character of that to which my invention relates, comprises the incorporation of wet nitrocellulose with 15 salts, formation into grains, preliminary drying, spraying with a solvent, and final drying. *Marshall on Explosives*, vol. I, page 324, sets forth this process with some particularity and specifies in detail the steps 20 that are usually practised. The wet nitrocellulose, which may be 40 per cent. water, is mixed with salts, which may be barium and potassium nitrates in known proportions. For example, the proportions may be 25 85 parts nitrocellulose calculated to the dry weight, 10 parts barium nitrate and five parts potassium nitrate. The ingredients are ground together in a mill, such as a wooden barrel with hard wood balls, or the 30 incorporation may be performed under edge runners similar to those used for the milling of black powder, as described by Marshall. The material is then passed through a sieve. The moist grains are, in the best practice, 35 spread on trays and dried by means of a current of hot air. The material is then allowed to cool. The necessary and important step of hardening, by treating with a solvent, is usually performed by spraying. Marshall 40 describes the known process of spraying the material while it is inside an hermetically closed rotary drum. The powder is then allowed to steep in the same vessel or in another one, and is subsequently dried.

45 The main objection to known processes, of which the foregoing described process is typical, resides in the hardening step of the process. The grains, after they are formed and dried, are tender and cannot stand much 50 friction. It is difficult or impossible to distribute the solvent uniformly. If too much solvent is received in one place, the grains coalesce into lumps. Again, if some of the 55 grains get little or no solvent, they remain mechanically unstable and are easily broken up in the subsequent handling or use of the

powder. With the best handling, lack of uniformity in the distribution of the solvent gives some difference in characteristics between the grains which have received more 60 solvent than they should and those which have not received as much as they should, making a product which is not quite uniform.

While my process involves, by preference, 65 some variation in detail in the grain-forming step, the essential feature of my process comprises a substantially new hardening or solvent-applying process whereby the difficulties and objections of known processes are 70 avoided. The invention will be best understood if I describe the operation, including known steps, in connection with the accompanying drawings, which are diagrams of the main apparatus, although it will be understood that my invention is not limited to 75 the employment of any particular mechanism.

Figure 1 is a sectional view of the incorporating drum. 80

Fig. 2 is a side elevation of the grain-forming apparatus.

Fig. 3 is a diagram of an apparatus which may be used in the hardening process.

The ingredients are incorporated in the 85 rotary drum *a* containing the hard wooden balls *b*. The material is then rubbed through a sieve *c* with meshes approximately the same as, or slightly larger than, the desired size of the grains. This sieve projects into 90 the end of a revolving cylinder *d*, which should be of considerable size, say thirty inches in diameter or more. This cylinder is open at both ends and slightly inclined. Upon rubbing the wet nitrocellulose mixture 95 through the sieve, particles fall down upon the revolving surface and are rolled immediately into grains, having a more or less round shape. This grained material then runs out from the other end of the cylinder, 100 and is dried in some kind of a drying apparatus which does not keep the grains in motion. An ordinary tray dry house will answer. The reason the material is not to be kept in motion, during drying, is that the 105 grains which have been formed when the nitrocellulose is wet would be disintegrated by friction upon one another after the material is dried.

The powder is now ready for the hardening process. I immerse the same completely in a mixture of a substance of relatively 110

high boiling point, which is a solvent of nitrocellulose, with a substance of relatively low boiling point, which is not a solvent of nitrocellulose. I use these two substances in such proportions that the mixture will not gelatinize nitrocellulose, or at least will not gelatinize it to an extent which will cause the grains to coalesce.

A preferred mixture is two parts by weight of carbon tetrachlorid (a non-solvent), which has a boiling point of about 76 degrees C., with one part of amyl acetate (a solvent), which has a boiling point of approximately 148 degrees C. These substances are perfectly miscible.

Having drained off the excess of the mixture, I then subject the grains to a recovery process in which a current of warm air passes over the mass while it is kept in motion. This I do in a revolving drum connected with a circulating fan, a heating coil and cooling coil, in a manner quite similar to that which has been applied to solvent recovery in the past. The apparatus shown in Fig. 3 will be effective. *f* represents the revolving drum, *g* the fan, *h* heating coils, *i* an outlet pipe from the drum, and *j* cooling coils.

What takes place in the recovery process is that the material of the lowest boiling point, or the non-solvent, which up to this time has interfered with the solvent acting upon the nitrocellulose, is driven off first, leaving the grains evenly moistened with the substance of higher boiling point, which is a solvent of nitrocellulose. In the example given, the carbon tetrachlorid is driven off first. At this point the colloidization of the nitrocellulose takes place and the grains are fixed. The recovery process then continues by the application of more heat, and the removal of the solvent proper takes place, leaving the grains finished.

By using the air circulating process, on account of the high vapor tension of both carbon tetrachlorid and amyl acetate, the recovery takes place at temperatures below the boiling points of these substances, so that

it is not necessary ever to heat the powder very hot in the recovery process. An initial heat of about 35 degrees C. raised gradually to about 60 degrees C. will suffice.

If there is a great difference between the boiling points of the two substances, as in the case of those mentioned, it is quite easy to separate them. Moreover, if the two substances, as in the examples given, have widely different specific gravities (carbon tetrachlorid 1.58, amyl acetate 0.866), the exact proportions of the mixture may be ascertained by determining its specific gravity, and thus may be corrected any errors of proportion in the recovered material that may have resulted from the loss of the more volatile ingredient.

Having now fully described my invention, what I claim and desire to protect by Letters Patent is:

1. The process of making smokeless shot gun nitrocellulose powder which comprises incorporating the ingredients, forming them into grains, treating them uniformly with a mixture of substances having different boiling points, one of which is a substance which, in a liquid condition at normal pressure and at a temperature below the ignition point of the nitrocellulose, is itself an active solvent of nitrocellulose but will not combine therewith to form a chemical compound, and the other of which is a liquid that is miscible with said solvent and not a solvent of the nitrocellulose, and then driving off the non-solvent, whereupon the nitrocellulose is colloidized and the grains are fixed.

2. The process of making smokeless shot gun nitrocellulose powder which comprises incorporating the ingredients, forming them into grains, treating them uniformly with a mixture of carbon tetrachlorid and amyl acetate, driving off the tetrachlorid to permit the amyl acetate to colloid the nitrocellulose, and then driving off the amyl acetate.

In testimony of which invention I have hereunto set my hand, at Wilmington, Delaware, on this 24th day of May, 1919.

FRANCIS I. DU PONT.